

May 4, 1954

H. H. MAYNES

2,677,496

BAG, COMPOSITE MATERIAL AND METHOD OF MAKING

Filed Sept. 22, 1950

FIG.1



FIG.2



FIG.3



INVENTOR:  
Harold H. Maynes  
BY *G. L. Deppendorff*

ATTORNEY

## UNITED STATES PATENT OFFICE

2,677,496

BAG, COMPOSITE MATERIAL, AND METHOD  
OF MAKINGHarold H. Maynes, Sparta, N. J., assignor to  
Arkell Safety Bag Company, New York, N. Y.,  
a corporation of New York

Application September 22, 1950, Serial No. 186,130

3 Claims. (Cl. 229—55)

1

The present invention relates to bags made of reinforced laminated or composite crinkled paper, and further relates to such composite material, and method of forming the same.

The object of the invention is to provide a novel and improved bag, composite material and method of this character.

The invention is illustrated, by way of example, in the accompanying drawings, in which:

Figure 1 is a diagrammatical side view, partly in section, of an apparatus that may be employed in carrying out my improved method;

Fig. 2 is a diagrammatical longitudinal sectional view of the composite material greatly enlarged; and

Fig. 3 is a side view, with one ply partly broken away, of my improved bag.

The composite material from which my improved bag is formed may be made of two sheets or webs 2 and 4, and a sheet or web of non-woven fabric 6 of fiber glass.

The paper sheets or webs 2 and 4 may be made of kraft or other strong crinkled paper. Preferably the crinkles extend generally transversely of the sheets and are of substantially the same stretchability. The degree of stretchability may be varied, but in making bags of the material I have obtained most satisfactory results with crinkled paper having approximately 6% to 8% stretchability. The crinkling is preferably formed by the water-crepe method which consists in passing each web to be crinkled through a water bath to a crinkling cylinder where it is removed by means of a doctor blade. By crinkling the sheets by the water-crepe method, it has been found that they have maximum elasticity.

The non-woven glass fabric 6 is made up of transverse and longitudinally extending yarns or threads 3 and 5, respectively, which are lightly secured together where they cross by asphaltic or other adhesive, the adhesive being applied by first running the longitudinal strands through the adhesive before the longitudinal and transverse strands are brought together one over the other. Any desired mesh may be employed such as 2 x 2 (1/2" mesh) and 4 x 4 (1/4" mesh), depending on the reinforcement, especially the tensile strength desired. The strands or threads may be relatively fine, corresponding substantially in diameter to ordinary six-cord cotton sewing thread, but the size of the threads may be varied to meet different conditions.

In forming the composite material, the crinkled webs 2 and 4 may be drawn from supply rolls 8, and the glass fabric 6 from a supply roll 10.

2

The paper webs with the glass fabric between them pass between two driven nip rolls 12. The upper web 2 passes over idlers 14 to the tip rolls and the lower web 4 passes over idlers 16 and between a coating roll 18 and a guide roll 20. The coating roll 18 receives asphaltic adhesive 22 from a metering and doctor roll 24, thus controlling the amount of adhesive applied to the web 4.

The adhesive in the pan 25 may be asphalt containing rubber or other elastomer so as to apply a more or less elastic coating to the web 4 which will remain tacky and elastic when set under varying atmospheric conditions. The coating applied to the web 4 is preferably thick enough to substantially fill the valleys between the crinkles as well as to cover the ridges of the crinkles.

As the glass fabric 6 passes with the paper webs between the nip rolls 12, the strands or threads of the fabric are forced down into the coating on the lower web 4 so as to be thoroughly embedded and covered thereby. The pressure of the nip rolls is such as to insure firm adherence of the crests of the crinkles of the web 2 to the web 4 and the threads of the fabric 6. Preferably the pressure of the nip rolls should not be sufficient to cause the coating to be forced materially into the valleys of the crinkles of the web 2.

When the two paper webs 2 and 4 and the reinforcing fabrics 6 have been thus brought together and the adhesive coating has become substantially set, the composite material may then be passed through a tubing machine, and the longitudinal edges of the material brought together in overlapping relation and glued to form the longitudinally extending seam 26. The tube as it is formed may be cut into bag lengths. The bag lengths may be closed at one end in any suitable manner as by means of a tape 28 folded over the end and held in place by adhesive or by adhesive and stitching to form the bottom of the bag. The other end of the bag may also be closed if desired and provided with a filling valve, or this end may be closed after filling the bag. The bag may have gusseted sides, or ungusseted sides as desired. Preferably the coated sheet of the bag forms the inner ply of the bag.

With the bag thus formed, the threads of the fabric are effectively cushioned by the elastic adhesive and the crinkled paper, so that in the use of the bag there is no danger of the threads being sharply bent or fractured. The adhesive surrounding and impregnating the twisted fibers of the threads tends to hold them together and strengthen them, and to keep the threads prop-

erly spaced. The dead air spaces provided between the valleys of the outer sheet and the adhesive coating cooperate to form a structure of cloth-like flexibility and of maximum strength. Thus the threads are not only thoroughly protected and reinforced by the crinkled paper and adhesive, but also during use of the filled bag the fabric, crinkled paper and adhesive are arranged most effectively to cooperate to resist bursting and other strains placed on the bag.

While it is preferred to coat only one of the webs in order to provide a light weight structure of maximum strength and flexibility, in certain instances the outer sheet may be either lightly coated to add to the moisture-proofness thereof without doing away with the air spaces between the valleys of the crinkles and the adhesive coating on the inner sheet, or a sufficient amount of adhesive may be applied to the outer sheet to substantially fill the valleys thereof.

What I claim is:

1. The method of forming composite material which comprises feeding at least two webs of crinkled paper longitudinally, the crinkles extending transversely of the webs, feeding a web of unwoven fabric longitudinally between said webs, said fabric web being composed of threads of glass fibers extending longitudinally thereof and spaced apart, and threads of glass fibers extending transversely thereof and spaced apart, applying a coating of tacky adhesive to the inner side of one of the paper webs as it is being fed with the adhesive filling the valleys and extending over the crinkles of said web, positioning the paper and fabric webs together under such pressure as to cause the threads of the fabric to be embedded in the adhesive and to cause the uncoated web to be secured only at the crests of its crinkles to the coated web so as to cause the

5 crinkles of the uncoated web to form air spaces between the webs.

2. Composite material of the class described comprising at least two webs of crinkled paper arranged in superposed relation with the crinkles extending transversely of the webs, a web of unwoven fabric arranged between said paper webs and composed of threads of glass fibers extending longitudinally thereof and spaced apart, and 10 threads of glass fibers extending transversely thereof and spaced apart, and tacky adhesive securing the webs together, the adhesive filling the valleys and extending over the crests of the crinkles of one of the paper webs with the threads of the fabric embedded in the adhesive, and the other web being secured by the adhesive only at the crests of the crinkles thereof so as to cause the valleys of the crinkles to form dead air spaces between the webs.

20 3. A bag made of the composite material of claim 2 with the crinkles thereof extending circumferentially of the bag.

#### References Cited in the file of this patent

#### UNITED STATES PATENTS

| Number       | Name      | Date           |
|--------------|-----------|----------------|
| 91,748       | Jameson   | June 22, 1869  |
| 1,197,315    | Wendler   | Sept. 5, 1916  |
| 1,821,824    | Woodward  | Sept. 1, 1931  |
| 30 1,867,071 | Collings  | July 12, 1932  |
| 1,870,215    | Anderson  | Aug. 9, 1932   |
| 1,871,827    | Van Hulst | Aug. 16, 1932  |
| 2,293,246    | Fay       | Aug. 18, 1942  |
| 35 2,314,876 | Greene    | Mar. 30, 1943  |
| 2,561,781    | Bruce     | July 24, 1951  |
| 2,610,936    | Carlson   | Sept. 16, 1952 |

#### FOREIGN PATENTS

| Number     | Country | Date         |
|------------|---------|--------------|
| 40 817,841 | France  | May 31, 1937 |